

# UNITED STATES PATENT OFFICE.

HENRY HOWARD GREENWAY, OF MELBOURNE, VICTORIA, AUSTRALIA, ASSIGNOR TO  
MINERALS SEPARATION LIMITED, OF LONDON, ENGLAND.

## CONCENTRATION OF ORES.

1,099,699.

Specification of Letters Patent.

Patented June 9, 1914.

No Drawing.

Application filed June 30, 1911. Serial No. 636,245.

To all whom it may concern:

Be it known that I, HENRY HOWARD GREENWAY, a subject of the King of England, residing at Melbourne, Victoria, Commonwealth of Australia, have invented certain new and useful Improvements in the Concentration of Ores, of which the following is a specification.

This invention relates to the concentration of ores and has been applied in practice to the concentration of copper ores the object being to separate certain constituents of the ore such as copper sulfids (for example in the form of copper pyrites) or metallic copper (natural or reduced) from other constituents such as gangue when the ore is suspended in a liquid such as water.

The present process is a modification of the invention described in U. S. patent to H. L. Sulman, A. H. Higgins and myself, No. 962,678, granted June 28, 1910. The process therein described is applicable generally to the recovery of metallic sulfids and like floatable metalliferous matter and in the case of lead and zinc sulfids to which the process has been largely applied it is necessary for efficient working that the pulp should be slightly acidified, and in most cases in practice the pulp is heated. It is now found that with copper ore such as an ore containing copper pyrites effective separation is obtained in the cold without the use of acid by employing as mineral frothing agents, aromatic hydroxy compounds such as phenol, cresol, or mixtures containing the same.

The process of concentrating ores containing copper sulfid or metallic copper according to this invention consists in mixing the powdered ore with water containing in solution a minute quantity of aromatic hydroxy compound such as phenol or cresol but without mineral acid and in the cold, agitating the mixture to form a froth and separating the froth. The hydroxy compounds may be used in the form of compounds containing them, such as wood tar oil which contains cresol; or if a mixture of hydroxy compounds is preferred, they may be used as a compound containing them such as Stockholm tar which contains substances of the phenol and cresol groups. If required there may be added to the water a small proportion of alkali to facilitate or effect the

solution of the aromatic hydroxy compound but it is important not to add such a quantity of alkali as will impair the formation or maintenance of the mineral bearing froth. The following is an example of one method of carrying this invention into effect. Water containing in solution a small quantity (in the examples hereinafter given 0.065% and 0.075%) of an aromatic hydroxy compound such as phenol or cresol or a mixture containing the same, is introduced with finely pulverized ore containing copper pyrites into an agitating apparatus in the proportion of say three or four parts by weight of water to one part by weight of ore. The agitation is carried out in such a way as to disseminate air through the mixture which is thereafter discharged into a spitzkasten. The operation is carried out in the cold and no acid is added to the pulp. It is found that coherent froth or scum floats on the surface of the water in the spitzkasten. This froth contains a large proportion of the metallic sulfid but is substantially free from gangue. Any well-known means may be employed for collecting the froth.

As an example of the results obtained in a process according to this invention cresol was used as a frothing agent, 1.45 lbs. per ton, in a neutral circuit at atmospheric temperature. The copper assay was as follows:

|                                  |                |
|----------------------------------|----------------|
| Ore                              | 2.45 per cent. |
| Concentrates obtained as a froth | 15.7 per cent. |
| Tailings                         | Trace          |

the results showing that the extraction was perfect.

In another case, using Stockholm tar, a substance containing a mixture of substances of the phenol and cresol groups, as the frothing agent, 1.67 lbs. per ton, under the same conditions as before, and on the same ore, the copper assay was as follows:

|              |                |
|--------------|----------------|
| Ore          | 2.5 per cent.  |
| Concentrates | 16.1 per cent. |
| Tailings     | 0.3 per cent.  |

the results showing that there was an extraction of 90 per cent.

What I claim as my invention and desire to secure by Letters Patent is:

1. A process of concentrating ores which consists in mixing a powdered ore with neu-

- tral water containing in solution a minute quantity of an aromatic hydroxy compound, agitating the mixture to form a froth and separating the froth.
- 5 2. A process of concentrating ores which consists in mixing a powdered ore with neutral water containing in solution a minute quantity of an aromatic hydroxy compound, agitating the mixture in the cold to form a 10 froth, and separating the froth.
3. A process of concentrating ores which consists in mixing a powdered ore containing copper with neutral water containing in solution a minute quantity of an aromatic 15 hydroxy compound, agitating the mixture to form a froth, and separating the froth.
4. A process of concentrating ores which consists in mixing a powdered ore containing copper with neutral water containing in 20 solution a minute quantity of an aromatic hydroxy compound, agitating the mixture in the cold to form a froth, and separating the froth.
5. A process of concentrating ores which 25 consists in mixing a powdered ore with neutral water containing in solution a minute quantity of a mixture of aromatic hydroxy compounds, agitating the mixture to form a froth, and separating the froth.
- 30 6. A process of concentrating ores which consists in mixing a powdered ore with neutral water containing in solution a minute quantity of a mixture of aromatic hydroxy compounds, agitating the mixture in the cold 35 to form a froth and separating the froth.
7. A process of concentrating ores which consists in mixing a powdered ore containing copper with neutral water containing in solution a minute quantity of a mixture of 40 aromatic hydroxy compounds, agitating the mixture to form a froth, and separating the froth.
8. A process of concentrating ores which 45 consists in mixing a powdered ore containing copper with neutral water containing in solution a minute quantity of a mixture of aromatic hydroxy compounds, agitating the mixture in the cold to form a froth, and separating the froth.
- 50 9. A process of concentrating ores which consists in mixing a powdered ore with neutral water containing in solution a minute
- quantity of cresol, agitating the mixture to form a froth, and separating the froth.
10. A process of concentrating ores which 55 consists in mixing a powdered ore with neutral water containing in solution a minute quantity of cresol, agitating the mixture in the cold to form a froth, and separating the froth.
11. A process of concentrating ores which 60 consists in mixing a powdered ore containing copper with neutral water containing in solution a minute quantity of cresol, agitating the mixture to form a froth, and separating the froth.
12. A process of concentrating ores which 65 consists in mixing a powdered ore containing copper with neutral water containing in solution a minute quantity of cresol, agitating the mixture in the cold to form a froth, and separating the froth.
13. A process of concentrating ores which 70 consists in mixing a powdered ore with neutral water containing in solution a minute quantity of wood tar oil, agitating the mixture to form a froth, and separating the froth.
14. A process of concentrating ores which 75 consists in mixing a powdered ore with neutral water containing in solution a minute quantity of wood tar oil, agitating the mixture in the cold to form a froth, and separating the froth.
15. A process of concentrating ores which 80 consists in mixing a powdered ore containing copper with neutral water containing in solution a minute quantity of wood tar oil, agitating the mixture to form a froth, and separating the froth.
16. A process of concentrating ores which 85 consists in mixing a powdered ore containing copper with neutral water containing in solution a minute quantity of wood tar oil, agitating the mixture in the cold to form a 90 froth, and separating the froth.
- 95 In testimony whereof I have signed my name to this specification in the presence of two subscribing witnesses.

HENRY HOWARD GREENWAY.

Witnesses:

J. M. MANGHAN,  
D. SEDDON.